

## UNITED STATES PATENT OFFICE

1,952,082

## ALLOY

Robert H. Leach, Fairfield, Conn., assignor to  
Handy & Harman, New York, N. Y., a corpora-  
tion of New York

No Drawing. Application June 10, 1932.  
Serial No. 616,498

3 Claims. (Cl. 75—1)

This invention relates to silver alloys and is concerned more particularly with a novel silver alloy which may be used to especial advantage in the manufacture of table silver and hollow 5 ware and for various other purposes, because it has the property of strongly resisting tarnish and discoloration.

As is well known, silver alloys of ordinary composition and containing copper as the base ingredient are susceptible to tarnish. Such discoloration of the metal is brought about by numerous agents, the most active being sulphur which is present in various foods such as eggs, and is also present to some extent in the atmosphere in the form of gaseous compounds. Sulphur in both forms causes tarnishing at a rate which depends on the length of contact or exposure of the metal, the concentration of the sulphur in the food or air, and the form in which 15 the sulphur is present. In any event, the necessity of frequent cleaning and polishing of silver articles to keep them in bright condition has led to numerous attempts in the past to produce silver alloys which are of good appearance, have 20 the desired working characteristics, and have a better resistance to tarnish than ordinary silver-copper alloys, but up to the present, the proposed alloys with which I am familiar, have not proven entirely satisfactory.

30 The problem of producing a silver alloy which is resistant to tarnish is a difficult one because investigation has shown that binary alloys offer little promise and the number of ternary and 35 quaternary alloys is very large. When it is understood that small variations in the ingredients in these alloys have an important effect on the resistance to tarnish and the amounts of the alloying ingredients used is highly critical with respect to tarnish resistance, the magnitude and 40 difficulty of the problem will be appreciated.

As a result of my investigations in this field, I have found that a silver alloy which has excellent resistance to tarnish produced by various causes may be made by using tin as an alloying metal, provided the amount of tin used be kept 45 within relatively narrow limits. The new alloy may be given a somewhat improved resistance to tarnish and, in some instances, better physical properties, if a small amount of a third ingredient 50 is used which is preferably chromium, although calcium may be substituted for chromium. This third ingredient has a slight hardening effect and, for convenience, it will be referred to as a "hardener", although it is to be understood that 55 it also increases the tarnish resistance to a substantial extent.

Silver alloys now in widest use are those of 60 sterling fineness and the new alloy of that fineness contains silver in an amount not less than about 92.5%, tin ranging from about 6% to about

7.1%, and, as a hardening ingredient, chromium in an amount ranging from about  $\frac{1}{4}$  up to about 1 $\frac{1}{2}$ %, or a similar amount of calcium replacing the chromium wholly or in part, chromium and calcium being substantially equivalent for the 65 purposes mentioned.

Typical examples of the new alloys in sterling fineness have the following approximate analyses:

|          | Example No. 1 | 70 |
|----------|---------------|----|
|          | Per cent      |    |
| Silver   | 92.5          |    |
| Tin      | 7.1           |    |
| Chromium | 0.4           | 75 |

|         | Example No. 2 | 75 |
|---------|---------------|----|
|         | Per cent      |    |
| Silver  | 92.5          |    |
| Tin     | 6.8           |    |
| Calcium | 0.7           | 80 |

I have found that chromium is the most satisfactory of the hardening ingredients that might be used and ordinarily the chromium employed need not exceed  $\frac{1}{2}$  of 1%. Also, while I have specified that the silver content shall be about 92.5%, it is to be understood that the silver may be increased in amount to some extent without impairing the quality of the new alloy.

I am aware that it has been proposed heretofore to employ tin and chromium, and tin and 90 nickel in silver alloys, but the alloys of this type with which I am familiar have contained less tin than the amounts specified above. A large number of experiments which I have conducted in this field have demonstrated that the range of 95 tin used in this alloy is quite critical and any departure from the range mentioned results in a lowering of the tarnish resistance, while within the specified range, the resistance is at its maximum.

## What I claim:

1. A silver alloy which consists of silver in the amount of about 92.5%, tin ranging from about 6% to about 7.1%, and chromium in an amount ranging from about 0.25% to about 1.5%.
2. A silver alloy which consists of about 92.5% silver, about 7.1% tin, and about 0.4% chromium.
3. A silver alloy which consists of silver in the amount of about 92.5%, tin ranging from about 6% to about 7.1%, and chromium in an amount 110 from about 0.25% to about 0.5%.

ROBERT H. LEACH.

115

120